



US009850590B2

(12) **United States Patent**  
**Hosokawa et al.**

(10) **Patent No.:** **US 9,850,590 B2**  
(45) **Date of Patent:** **Dec. 26, 2017**

(54) **ANODIZED ALUMINUM FILM**(71) Applicant: **Kobe Steel, Ltd.**, Kobe-shi (JP)(72) Inventors: **Mamoru Hosokawa**, Kobe (JP);  
**Satoru Takada**, Kobe (JP)(73) Assignee: **Kobe Steel, Ltd.**, Kobe-shi (JP)

(\* ) Notice: Subject to any disclaimer, the term of this patent is extended or adjusted under 35 U.S.C. 154(b) by 64 days.

(21) Appl. No.: **14/418,262**(22) PCT Filed: **Sep. 24, 2013**(86) PCT No.: **PCT/JP2013/075662**

§ 371 (c)(1),

(2) Date: **Jan. 29, 2015**(87) PCT Pub. No.: **WO2014/050794**PCT Pub. Date: **Apr. 3, 2014**(65) **Prior Publication Data**

US 2015/0211141 A1 Jul. 30, 2015

(30) **Foreign Application Priority Data**

Sep. 26, 2012 (JP) ..... 2012-212732

(51) **Int. Cl.**

**C25D 11/04** (2006.01)  
**C25D 11/06** (2006.01)  
**C25D 11/12** (2006.01)  
**C25D 11/08** (2006.01)  
**C25D 11/10** (2006.01)

(52) **U.S. Cl.**

CPC ..... **C25D 11/04** (2013.01); **C25D 11/06** (2013.01); **C25D 11/12** (2013.01); **C25D 11/08** (2013.01); **C25D 11/10** (2013.01)

(58) **Field of Classification Search**

None

See application file for complete search history.

(56) **References Cited**

## U.S. PATENT DOCUMENTS

4,606,796 A \* 8/1986 Hanazima ..... C25D 11/18  
205/174  
5,277,788 A \* 1/1994 Nitowski ..... C25D 11/12  
205/172

6,027,629 A 2/2000 Hisamoto et al.  
2008/0213618 A1 \* 9/2008 Critchlow ..... C25D 11/08  
428/613

2012/0132529 A1 5/2012 Zekry et al.  
2012/0256224 A1 10/2012 Hatanaka et al.

## FOREIGN PATENT DOCUMENTS

|    |               |          |
|----|---------------|----------|
| CN | 101962792 A   | 2/2011   |
| JP | 8 193295      | 7/1996   |
| JP | 10138034 A    | * 5/1998 |
| JP | 2004001171 A  | * 1/2004 |
| JP | 2011-117042 A | 6/2011   |
| JP | 2011 132586   | 7/2011   |
| JP | 2011 157624   | 8/2011   |
| JP | 2012-117144 A | 6/2012   |
| JP | 2012-162769 A | 8/2012   |

## OTHER PUBLICATIONS

Hideki Masuda, et al., "Process to make anodic oxidation coating on aluminum thick—Produce a film having a thickness of 2 mm" Proceedings of ARS Conference, Oct. 1992, 4 Pages (with English translation).

International Search Report and Written Opinion of the International Searching Authority Issued Dec. 17, 2013 in PCT/JP13/075662 Filed Sep. 24, 2013.

\* cited by examiner

*Primary Examiner* — Vera Katz(74) *Attorney, Agent, or Firm* — Oblon, McClelland, Maier & Neustadt, L.L.P.(57) **ABSTRACT**

Provided is an anodized aluminum film formed on a surface of a substrate that comprises aluminum or an aluminum alloy, the anodized aluminum film having a structure constituted of a single anodized film layer or a structure composed of superposed anodized film layers of two or more different kinds, wherein the outermost anodized film has a degree of film formation, defined by equation (1), of 1.3 or more and the proportion of the thickness of this anodized film in the entire film thickness is 3% or higher. Thus, the anodized aluminum film is inhibited from cracking in bent portions. As a result, the substrate is inhibited from corroding in corrosive-gas atmospheres, and a decrease in withstand voltage characteristics due to film cracking is inhibited. With this anodized aluminum film, enhanced withstand voltage characteristics can hence be attained:

Degree of film formation=(thickness of anodized film)/(substrate thickness loss by anodization) (1).

**11 Claims, No Drawings**

**1**  
**ANODIZED ALUMINUM FILM**

TECHNICAL FIELD

The present invention relates to an anodized aluminum film preferably used for an aluminum member having an anodized film on a substrate of aluminum alloy useful as a material for a vacuum chamber of manufacturing equipment of semiconductor or liquid crystal, the equipment including a dry etching apparatus, a chemical vapor deposition (CVD) apparatus, an ion implantation apparatus, and a sputtering apparatus, or useful as a material of a component provided within the vacuum chamber. In particular, the invention relates to an anodized aluminum film that is improved in withstand voltage characteristics while cracking is suppressed in a curved portion.

BACKGROUND ART

There has been widely practiced anodizing that forms an anodized film on a surface of a member including a substrate of aluminum, aluminum alloy, or the like to improve plasma resistance and gaseous corrosion resistance of the substrate. For example, a vacuum chamber used in a plasma treatment apparatus of semiconductor manufacturing equipment or each of various components provided within the vacuum chamber is typically composed of aluminum alloy. However, if the aluminum alloy is used while being untreated (solid), its properties such as plasma resistance and gaseous corrosion resistance cannot be maintained. An anodized film is therefore provided on a surface of the member composed of aluminum alloy to improve plasma resistance, gaseous corrosion resistance, and the like.

In recent years, power to be applied for plasma generation increases with increase in plasma density due to narrowed interconnection width. In existing anodized films, therefore, dielectric breakdown may be induced by high temperature and high voltage occurring at high power application. Electric properties of the film are varied in a portion where such dielectric breakdown occurs, and therefore the film is less uniformly etched or formed in the portion. The anodized film is therefore desired to be improved in crack resistance and withstand voltage characteristics.

Various techniques have been previously proposed in order to improve properties of the anodized film. For example, PTL 1 suggests that pore size on a surface side of an anodized film is controlled to be small on a side near a film surface and large on a side near a substrate, thereby the anodized film is reduced in reactivity to plasma so as to improve plasma resistance. Such an anodized film can be extremely improved in plasma resistance compared with existing anodized films. In such an anodized film, however, cracking (hereinafter sometimes referred to as "curved-portion cracking") may also occur in a curvature portion (curved portion) that may exist in actual equipment. This may lead to an environment under which the substrate and the anodized film are each easily corroded.

CITATION LIST

Patent Literature

PTL 1: Japanese Unexamined Patent Application Publication No. Hei8 (1996)-193295.

**2**

SUMMARY OF INVENTION

Technical Problem

5 An object of the invention, which has been made in light of the above-described circumstances, is to provide an anodized aluminum film that is improved in withstand voltage characteristics by suppressing curved-portion cracking and therethrough suppressing corrosion of a substrate under corrosive gas atmosphere and degradation in withstand voltage characteristics due to film cracking.

Solution to Problem

15 According to the present invention, there is provided an anodized aluminum film, by which the object is achieved, formed on a surface of a substrate including aluminum or aluminum alloy, the anodized aluminum film including an anodized film having a monolayer film structure or at least 20 two laminated anodized films having different film structures, a top-side anodized film having a degree of film formation of 1.3 or more, the degree of film formation being defined by Formula (1), and having a thickness percentage of 3% or more relative to the entire film thickness.

25

$$\text{Degree of film formation} = (\text{thickness of anodized film}) / (\text{substrate thickness loss by anodization}) \quad (1)$$

The anodized aluminum film of the invention preferably has a smaller thickness of the entire film in light of suppressing cracking, but extremely small thickness thereof anxiously leads to degradation in corrosion resistance; hence, the total thickness should be, for example, 3  $\mu\text{m}$  or more. The entire film thickness is preferably 20  $\mu\text{m}$  or more (more preferably 25  $\mu\text{m}$  or more) in light of maintaining withstand voltage characteristics. The entire film thickness refers to thickness of one film for a monolayer film structure, and refers to the total film thicknesses of respective layers for a multilayer film structure including at least two laminated anodized films having different film structures.

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

5290

5295

5300

5305

5310

5315

5320

5325

5330

5335

5340

5345

5350

5355

5360

5365

5370

5375

5380

5385

5390

5395

5400

5405

5410

5415

5420

5425

5430

5435

5440

5445

5450

5455

5460

5465

5470

5475

inventors have found that when at least a top-side anodized film is formed such that the degree of film formation defined by the predetermined relational expression is 1.3 or more, and when thickness of the top-side anodized film is defined to be within a predetermined range, an anodized film, which enables the above-described object to be achieved, is given, and finally they have completed the invention.

It is considered that cracking basically occurs in a curved portion when volume loss (i.e., thickness loss) of a substrate by anodizing is not sufficiently filled with the anodized film to be formed. The anodized film is therefore designed to have a degree of film formation of 1.3 or more, the degree of film formation being defined by Formula (1), thereby the volume loss of the substrate can be filled with the anodized film, and the curved-portion cracking can be suppressed. Although the degree of film formation of 1.0 or more is considered to be high enough to fill the volume loss of the substrate with the anodized film, such an anodized film has failed to achieve the object. In other words, the object has been achieved only by the anodized film having the degree of film formation of 1.3 or more.

One possible reason why such a phenomenon occurs is estimated to be that the anodized film having the degree of film formation of 1.3 or more is easily stretched due to a variation in structure (internal film structure) of the film itself, and thus the film is increased in stretch rate to a stress applied on the film, and consequently the curved-portion cracking is less likely to occur.

The degree of film formation is preferably 1.5 or more, more preferably 1.7 or more, and further preferably 2.0 or more. The degree of film formation can be adjusted by appropriately controlling a condition of the anodizing (as described later). However, if treatment time is increased, a surface of the anodized film is dissolved in a treatment solution, and thickness of the film is decreased; hence, the degree of film formation is limitedly increased up to a certain value. The upper limit of the degree of film formation is typically about 3.

In light of suppressing the curved-portion cracking, thickness of an anodized film having a degree of film formation of 1.3 or more (such a film may be referred to as "top-side film") is preferably 3% or more in percentage to the entire film thickness. It is preferred that the entire film thickness is specifically 3  $\mu\text{m}$  or more.

The anodized film of the invention includes the following two cases, i.e., a case where a film structure (laminated film structure) is a monolayer structure, and a case where the film structure is a multilayer structure including at least two layers having different film structures. For the monolayer, the anodized film has a thickness percentage of 100% relative to the entire film thickness, and the preferable lower limit, 3  $\mu\text{m}$  or more, of the entire film thickness corresponds to thickness of one layer. A substrate-side anodized film also has a degree of film formation of 1.3 or more.

In the withstand voltage characteristics to be required, withstand voltage of the anodized film as a whole (or withstand voltage of a planar portion) is preferably 600 V or more (more preferably 1000 V or more, and further preferably 1500 V or more). Since withstand voltage characteristics of the anodized film as a whole is in proportion to film thickness for the same film structure, the entire film thickness (total thickness) is preferably 20  $\mu\text{m}$  or more in order to maintain good withstand voltage characteristics. The entire film thickness is more preferably 25  $\mu\text{m}$  or more (further preferably 30  $\mu\text{m}$  or more, and most preferably 40  $\mu\text{m}$  or more). However, if the entire film thickness is increased, the film is easily cracked due to internal stress of

the film, and withstand voltage is rather lowered; hence, the total thickness is preferably 200  $\mu\text{m}$  or less (more preferably 100  $\mu\text{m}$  or less).

The anodized film (top-side film) having a degree of film formation of 1.3 or more tends to be increased in leakage current during measurement of withstand voltage. If the leakage current increases, a feeble current may flow through the film while not lead to film breakage caused by dielectric breakdown. This tends to cause a problem such as plasma abnormal discharge in a semiconductor process, for example.

The inventors have also made investigations in light of solving such a problem. As a result, it has been found that since leakage current is less likely to occur in the anodized film having a degree of film formation of less than 1.3 (such a film may be referred to as "substrate-side film"), if such a film is provided on a substrate side, leakage current can be inhibited.

Specifically, the anodized film is designed to have a film structure (laminated film structure) where the anodized film having a degree of film formation of less than 1.3 is provided on the substrate side, and the anodized film having a degree of film formation of 1.3 or more is provided on the top side, thereby crack resistance can be suppressed, and leakage current can be decreased. When such a laminated film structure is used, thickness of the substrate-side film is preferably 10% or more (i.e., thickness of the top-side film is 90% or less), more preferably 20% or more (further preferably 30% or more), relative to the entire film thickness in order to effectively allow the above-described effects to be exhibited.

When the anodized film of the invention includes at least two laminated layers having different film structures, and if at least the requirement for the anodized film provided on each of the top side and the substrate side is satisfied, the object of the invention can be achieved. However, this is not intended to limit the film structure (laminated film structure) of the anodized film of the invention to the two-layer structure. The film structure may include a three-layer structure and a four-layer structure as long as such requirements are satisfied. However, if the number of such laminated layers is excessively large, the treatment process is complicated, and the effects are not further effectively exhibited; hence, the number is appropriately up to four.

The at least two anodized films having different film structures should be prepared with different treatment solutions or treatment conditions (described later) for formation of the anodized films.

The anodized film having a degree of film formation of 1.3 or more should be basically formed through increasing temperature of a treatment solution, and decreasing a treatment voltage or current density depending on a type of an anodizing solution (electrolytic solution) to be used. Specifically, when oxalic acid is used as the treatment solution, temperature of the treatment solution (solution temperature) is preferably about 20 to 30  $^{\circ}\text{C}$ .

The voltage (electrolysis voltage) during anodizing is preferably about 30 to 60 V (more preferably 35 to 55 V). Alternatively, the current density of a current applied during anodizing is preferably 1.0 A/dm<sup>2</sup> or less (more preferably 0.8 A/dm<sup>2</sup> or less, further preferably 0.6 A/dm<sup>2</sup> or less). However, such specific conditions may be appropriately adjusted depending on a type of the treatment solution (the treatment solution composition) or a type of the substrate (including aluminum or aluminum alloy).

By contrast to such a condition, the anodized film having a degree of film formation of less than 1.3 should be

basically formed through relatively decreasing temperature of the treatment solution (to about 10 to 20° C.), and increasing a treatment voltage or current density. Specifically, when oxalic acid is used as the treatment solution, the voltage (electrolysis voltage) during anodizing is preferably about 60 to 80 V (more preferably about 70 to 80 V). The current density of a current applied during anodizing preferably has a value larger than 1.0 A/dm<sup>2</sup> (more preferably 1.4 A/dm<sup>2</sup> or more).

The anodizing solution usable in the invention includes not only the above-described oxalic acid, but also, for example, organic acid such as formic acid, inorganic acid such as phosphoric acid, chromic acid, and sulfuric acid, and mixed acids thereof. The concentration of the anodizing solution should be appropriately controlled such that desired functions and effects are effectively exhibited. For example, the concentration is preferably controlled to be about 1 to 5% for oxalic acid.

The substrate used in the invention is composed of aluminum or aluminum alloy. Any type of aluminum or aluminum alloy, which is typically used for formation of an anodized film, may be used without limitation. For example, any of aluminum alloys of 1000 series (industrial pure Al), 5000 series, and 6000 series can be used. A commercially available aluminum alloy may also be used as the aluminum alloy.

The anodized film of the invention is decreased in cracking in a curved portion and improved in withstand voltage characteristics; hence, the anodized film can be preferably used for a vacuum chamber of manufacturing equipment of semiconductor or liquid crystal, or components provided within the vacuum chamber, such as a clammer, a shower head, and a susceptor. The anodized film of the invention may also be subjected to sealing such as boiling water sealing or pressurized-steam sealing in order to improve acid resistance in a wet process.

Although the invention is now described in detail with an example, the invention should not be limited thereto, and modifications or alterations thereof may be made within the scope without departing from the gist described before and later, all of which are included in the technical scope of the invention.

This application claims the benefit of Japanese Priority Patent Application JP 2012-212732 filed on Sep. 26, 2012, the entire contents of which are incorporated herein by reference.

## EXAMPLE

A rolled material (base material) of 6061 alloy defined by JIS H 4000 was used as an aluminum alloy substrate, and a plurality of test specimens each having a size of 25 mm wide, 35 mm long (in a rolling direction), and 2 mm thick were cut out from the rolled material and were subjected to facing.

Subsequently, each of the specimens was anodized under a condition (including a treatment solution type, treatment solution temperature, and electrolysis voltage or electrolysis current density) shown in Table 1, and thus anodized films having various film structures (monolayer or multilayer) were prepared.

The degree of film formation, film thickness, and total thickness of each anodized film were measured according to the following procedures. Table 1 collectively shows results of such measurements.

## 25 (Measurement of Degree of Film Formation and Thickness of Anodized Film)

Part of a surface of the substrate was masked, and then the surface was anodized to form an anodized film. The resultant specimen was embedded in resin and polished, and was then observed along a film section direction by a light microscope. A position of the Al alloy in the masked portion was defined as an original substrate position, and a distance from the original substrate position to a substrate position in the portion where the anodized film was formed was defined as substrate thickness loss. Film thickness (i.e., thickness of each layer and total thickness) was measured through observation along the film section direction. The degree of film formation was obtained through calculation according to Formula (1) using the measured thicknesses. The measurement was performed in five portions in total, and the average of the measured values was obtained.

TABLE 1

| Test No. | Treatment solution type            | Treatment solution temperature (° C.) | Electrolysis voltage (V) | Electrolysis current density (A/dm <sup>2</sup> ) | Degree of film formation (—) | Film structure<br>Top-side film           |                |                                                      | Determination of thickness |
|----------|------------------------------------|---------------------------------------|--------------------------|---------------------------------------------------|------------------------------|-------------------------------------------|----------------|------------------------------------------------------|----------------------------|
|          |                                    |                                       |                          |                                                   |                              | Determination of degree of film formation | Thickness (μm) | Thickness percentage relative to total thickness (%) |                            |
| 1        | 5% oxalic acid                     | 30                                    | 40                       | —                                                 | 2.3                          | ○                                         | 2              | 18                                                   | ○                          |
| 2        | 5% oxalic acid                     | 30                                    | —                        | 0.8                                               | 2.3                          | ○                                         | 5              | 20                                                   | ○                          |
| 3        | 4% oxalic add + 0.3% sulfuric add  | 13                                    | 60                       | —                                                 | 2.3                          | ○                                         | 2              | 7                                                    | ○                          |
| 4        | 4% oxalic add + 0.3% sulfuric add  | 13                                    | 60                       | —                                                 | 2.3                          | ○                                         | 19             | 38                                                   | ○                          |
| 5        | 4% oxalic add + 0.3% sulfuric add  | 13                                    | 60                       | —                                                 | 2.3                          | ○                                         | 10             | 25                                                   | ○                          |
| 6        | 4% oxalic acid                     | 20                                    | 40                       | —                                                 | 1.4                          | ○                                         | 3              | 16                                                   | ○                          |
| 7        | 4% oxalic acid                     | 25                                    | 40                       | —                                                 | 2.2                          | ○                                         | 11             | 100                                                  | ○                          |
| 8        | 3% oxalic acid                     | 30                                    | —                        | 0.7                                               | 2.1                          | ○                                         | 26             | 100                                                  | ○                          |
| 9        | 3% oxalic acid                     | 28                                    | 35                       | —                                                 | 1.7                          | ○                                         | 22             | 88                                                   | ○                          |
| 10       | 3% oxalic add + 0.1% sulfuric acid | 13                                    | 50                       | —                                                 | 2.3                          | ○                                         | 2              | 18                                                   | ○                          |
| 11       | 5% oxalic acid                     | 17                                    | —                        | 1.4                                               | 1.2                          | X                                         | 27             | 100                                                  | ○                          |
| 12       | 3% oxalic acid                     | 17                                    | 80                       | —                                                 | 1.1                          | X                                         | 50             | 100                                                  | ○                          |

TABLE 1-continued

| 13                  | 3% oxalic acid                           | 30                       | 40                                   | —              | 2.1                          | ○                    | 1 | 2  | X |
|---------------------|------------------------------------------|--------------------------|--------------------------------------|----------------|------------------------------|----------------------|---|----|---|
| 14                  | 3% oxalic<br>add + 0.1%<br>sulfuric acid | 13                       | 50                                   | —              | 2.3                          | ○                    | 1 | 2  | X |
| 15                  | 2% oxalic acid                           | 17                       | 70                                   | —              | 1.2                          | X                    | 3 | 43 | ○ |
| Film structure      |                                          |                          |                                      |                |                              |                      |   |    |   |
| Substrate-side film |                                          |                          |                                      |                |                              |                      |   |    |   |
| Test No.            | Treatment solution temperature (° C.)    | Electrolysis voltage (V) | Electrolysis current density (A/dm²) | Thickness (μm) | Degree of film formation (—) | Total thickness (μm) |   |    |   |
| 1                   | 17                                       | 80                       | —                                    | 9              | 1.2                          | 11                   |   |    |   |
| 2                   | 17                                       | —                        | 1.4                                  | 20             | 1.2                          | 25                   |   |    |   |
| 3                   | 10                                       | 60                       | —                                    | 20             | 1.1                          | 22                   |   |    |   |
| 4                   | 17                                       | 70                       | —                                    | 30             | 1.1                          | 49                   |   |    |   |
| 5                   | 17                                       | 70                       | —                                    | 30             | 1.1                          | 40                   |   |    |   |
| 6                   | 10                                       | 60                       | —                                    | 16             | 1.1                          | 19                   |   |    |   |
| 7                   | —                                        | —                        | —                                    | 0              | —                            | 11                   |   |    |   |
| 8                   | —                                        | —                        | —                                    | 0              | —                            | 26                   |   |    |   |
| 9                   | 18                                       | —                        | 1.3                                  | 3              | 1.1                          | 25                   |   |    |   |
| 10                  | 10                                       | 60                       | —                                    | 9              | 1.2                          | 11                   |   |    |   |
| 11                  | —                                        | —                        | —                                    | 0              | —                            | 27                   |   |    |   |
| 12                  | —                                        | —                        | —                                    | 0              | —                            | 50                   |   |    |   |
| 13                  | 17                                       | 80                       | —                                    | 40             | 1.1                          | 41                   |   |    |   |
| 14                  | 10                                       | 60                       | —                                    | 40             | 1.2                          | 41                   |   |    |   |
| 15                  | 18                                       | 70                       | —                                    | 4              | 1.0                          | 7                    |   |    |   |

For each of the anodized films (Test Nos. 1 to 15), occurrence of curved-portion cracking was evaluated, and withstand voltage and leakage current were measured. Table 2 shows results of them.

#### (Evaluation of Occurrence of Curved-Portion Cracking)

With the curved-portion cracking, occurrence of curved-portion cracking was observed along a film surface direction by a light microscope with 100 $\times$  and 200 $\times$  magnifications in a curved portion (a portion with R of 2 mm) of each test specimen. In the case where a distinct crack existed in the film surface, crack resistance was determined to be bad ("x" in Table 2). In the case where no crack was viewed, crack resistance was determined to be good ("○" in Table 2).

#### (Measurement of Withstand Voltage and Leakage Current)

The withstand voltage and leakage current of each specimen were determined as follows. For the withstand voltage, a withstand voltage tester ("TOS5051A" from KIKUSUI ELECTRONICS CORPORATION) was used in such a manner that a plus terminal was connected to a needle probe and was vertically brought into contact with the anodized film (a planar portion), a minus terminal was connected to the aluminum alloy substrate, a voltage was applied, and the withstand voltage characteristics were determined by a dielectric breakdown voltage (referred to as "planar-portion withstand voltage"). The leakage current in the planar portion (planar-portion leakage current) was measured in the same way. In each of Test Nos. 1 to 10, the planar-portion withstand voltage was 600 V or higher.

TABLE 2

| Test No. | Evaluation of film      |                                     |
|----------|-------------------------|-------------------------------------|
|          | Curved-portion cracking | Planar-portion leakage current (mA) |
| 1        | ○                       | 0.01                                |
| 2        | ○                       | 0.01                                |

TABLE 2-continued

| Test No. | Evaluation of film      |                                     |
|----------|-------------------------|-------------------------------------|
|          | Curved-portion cracking | Planar-portion leakage current (mA) |
| 3        | ○                       | 0.03                                |
| 4        | ○                       | 0.01                                |
| 5        | ○                       | 0.01                                |
| 6        | ○                       | 0.03                                |
| 7        | ○                       | 0.04                                |
| 8        | ○                       | 0.05                                |
| 9        | ○                       | 0.02                                |
| 10       | ○                       | 0.02                                |
| 11       | X                       | 0.02                                |
| 12       | X                       | 0.02                                |
| 13       | X                       | 0.03                                |
| 14       | X                       | 0.02                                |
| 15       | X                       | 0.03                                |

The following consideration can be made from such results. Test Nos. 1 to 10 are examples that each satisfy the requirements defined in the invention, in each of which curved-portion cracking does not occur, and good withstand voltage characteristics (low leakage current) are shown. Each of Test Nos. 7 and 8 is an example having no second layer, showing a slightly high value of the leakage current.

In contrast, each of Nos. 11 to 15 is a comparative example that does not satisfy at least one of the requirements defined in the invention, and is degenerated in at least one of properties. Among them, Test Nos. 11 and 12 are each a comparative example having the first layer (top-side layer) configured of an anodized film having a degree of film formation of less than 1.3 and having no second layer, in which the withstand voltage characteristics are good in the planar portion having no crack, but the withstand voltage of the anodized film as a whole is expected to be low because curved-portion cracking occurs.

In each of Test Nos. 13 and 14, a thickness percentage of the top-side film is insufficiently small, and curved-portion

cracking occurs. Test No. 15 is an example having a top-side film configured of an anodized film having a degree of film formation of less than 1.3, showing curved-portion cracking.

## INDUSTRIAL APPLICABILITY

In the invention, the top-side anodized film has a degree of film formation of 1.3 or more, the degree of film formation being defined by Formula (1), and has a thickness percentage of 3% or more relative to the entire film thickness, thereby the curved-portion cracking is suppressed, so that corrosion of a substrate under corrosive gas atmosphere and degradation in withstand voltage characteristics due to film cracking are suppressed, and consequently an anodized aluminum film having excellent withstand voltage characteristics is produced:

$$\text{Degree of film formation} = (\text{thickness of anodized film}) / (\text{substrate thickness loss by anodization}) \quad (1)$$

The invention claimed is:

1. An anodized aluminum film formed on an anodized surface of a substrate comprising aluminum or an aluminum alloy, wherein the anodized aluminum film is formed within a thickness loss of the substrate resulted from anodizing, wherein the anodized aluminum film is an anodized film having at least three laminated anodized films having different film structures, wherein a top-side anodized film of the at least two laminated anodized films has a degree of film formation of 1.3 or more, wherein the degree of film formation is defined by the following Formula:

$$\text{Degree of film formation} = (\text{thickness of top-side anodized film}) / (\text{substrate thickness loss by anodization}),$$

and wherein the top-side anodized film has a thickness percentage of 3% or more relative to a total anodized aluminum film thickness, thereby suppressing a curve portion cracking.

2. The anodized aluminum film according to claim 1, wherein the total anodized aluminum film thickness is 3  $\mu\text{m}$  or more.

5 3. The anodized aluminum film of claim 2, wherein the at least three anodized films having different film structures are prepared with different treatment solutions or different treatment conditions.

10 4. The anodized aluminum film of claim 2, wherein the total anodized aluminum film thickness is 20  $\mu\text{m}$  or more.

5 5. The anodized aluminum film according to claim 1, wherein the at least three anodized films having different film structures are prepared with different treatment solutions or different treatment conditions.

15 6. The anodized aluminum film of claim 5, wherein the at least three anodized film having different film structures are prepared with different treatment solutions.

20 7. The anodized aluminum film of claim 6, wherein at least one of the different treatment solutions comprises an acid.

25 8. The anodized aluminum film of claim 6, wherein at least one of the different treatment solutions comprises an acid selected from the group consisting of an organic acid, an inorganic acid, and a mixture thereof.

30 9. The anodized aluminum film of claim 6, wherein at least one of the different treatment solutions comprises at least one selected from the group consisting of oxalic acid, formic acid, phosphoric acid, chromic acid and sulfuric acid.

35 10. The anodized aluminum film of claim 1, wherein the substrate comprises the aluminum alloy.

11. The anodized aluminum film of claim 10, wherein the aluminum alloy is selected from the group consisting of a 1000 series aluminum alloy, a 5000 series aluminum alloy, and a 6000 series aluminum alloy.

\* \* \* \* \*